

75-84 XR

Patented Nov. 17, 1925.

1,562,201

## UNITED STATES PATENT OFFICE.

JOHN J. BOERICKE, OF MERION, PENNSYLVANIA.

## METHOD OF PRODUCING MOLYBDENUM AND VANADIUM ALLOYS.

No Drawing. Application filed May 26, 1920, Serial No. 384,311. Renewed September 25, 1925.

*To all whom it may concern:*

Be it known that I, JOHN J. BOERICKE, a citizen of the United States, residing at Merion, in the county of Montgomery and 5 State of Pennsylvania, have invented certain new and useful Improvements in Methods of Producing Molybdenum and Vanadium Alloys, of which the following is a specification.

10 This invention relates to a process for producing molybdenum and vanadium alloys such as used for the making of alloy steels, for example. As instances of such alloys, I mention ferro-molybdenum and 15 ferro-vanadium, the percentage of molybdenum and vanadium, respectively, being relatively high as compared with the alloying metal.

It is one of the primary objects of my 20 invention to increase the yield of such high percentage molybdenum and vanadium alloys.

In carrying out my invention I prepare an alumino-thermic mixture of the molybdenum or vanadium compound employed as source of one of these metals for the alloy, as the case may be, and aluminum, together with a relatively large quantity of a flux such as lime, or fluor-spar, and the alloying 25 metal. This alumino-thermic mixture is reduced by any preferred alumino-thermic process.

I am aware that it is old in this art to use fluxes such as lime, fluor-spar and the 30 like in the reduction of the rarer metals, and also that it is old to produce high percentage tungsten alloys with a large percentage of such a flux. In the latter case, however, the large quantity of such flux is 35 added because of the high fusion temperature of the tungsten, in which and other respects, molybdenum and vanadium are quite different from tungsten. It was not to be expected, therefore, that with respect 40 to molybdenum and vanadium, the use of a large quantity of such a flux, which is indifferent in that it does not raise the reaction temperature, would produce any useful result not obtainable with the ordinary 45 amount of flux used in the reduction of 50

molybdenum and vanadium in standard alumino-thermic practices. I have discovered, however, that with a large quantity of flux in the mixture the proportionate yield of alloy from its reduction is increased. 55 In a normal combination there is a certain expected theoretical or natural quantity or percentage of flux but I prefer to use an additional quantity of flux the amount of which is roughly equivalent to this theoretical or natural percentage. 60

Instead of adding the flux as a separate component part of the mixture, the process may be carried out with a compound wherein the flux is combined with the metal in 65 the natural state as, for example, calcium molybdate.

Simply by way of example I have found that where a reduction is carried out involving the use of say roughly 200 pounds of 70 calcium molybdate it is advisable to use approximately 25 pounds of slacked lime in addition. This is given only as one general example as there may be a great number of variations in the amount of the excess flux 75 used but I have found that the above will increase the yield from 15 to 20% or thereabouts.

I claim:

1. The herein described process of producing high percentage alloys of molybdenum or vanadium which consists in reducing an alumino-thermic mixture consisting of the molybdenum or vanadium compound, the alloying metal, a reducing metal, 85 and a quantity of indifferent flux materially in excess of that for the purposes of standard alumino-thermic practices.

2. The herein described process of producing high percentage alloys of molybdenum 90 or vanadium which consists in reducing an alumino-thermic mixture consisting of the molybdenum or vanadium compound, the alloying metal, a reducing metal, and a quantity of flux which is roughly twice the 95 amount theoretically calculated upon.

In testimony whereof, I have hereunto signed my name.

JOHN J. BOERICKE.